

April 28, 1942.

C. A. LAISE

2,281,446

ELECTRICAL CONTACT

Filed Jan. 7, 1937

Fig. 1.



Fig. 2.



Fig. 3.



Fig. 4.



INVENTOR.  
Clemens A. Laise  
BY *Charles Holland*  
ATTORNEY.

## UNITED STATES PATENT OFFICE

2,281,446

## ELECTRICAL CONTACT

Clemens A. Laise, Tenafly, N. J.; Fidelity Union Trust Company, executor of said Clemens A. Laise, deceased, assignor to Callite Tungsten Corporation, Union City, N. J., a corporation of Delaware

Application January 7, 1937, Serial No. 119,378

13 Claims. (Cl. 200—166)

This invention relates to the art of composite metal bodies and is particularly concerned with such bodies in the form of sheets or plates, composed of three metals or metal alloys, adapted to be cut, punched, stamped, extruded or drawn out into a shape suitable for use as face plates for electrical contacts.

The invention contemplates the construction of electrical contacts in which the metal which serves actually to make the contact which completes an electrical circuit, is composed of silver or silver alloy.

The invention is applicable to electrical contacts of various types and to vibratory circuit-making and -breaking devices of the type adapted for use as sparking or igniting contacts for internal combustion engines, circuit controllers, regulators, therapeutic apparatus, automatic recording machines, sign flashers, etc.

Heretofore, silver contacts have been made in the form of a face plate welded to a base of brass or cuprous metal in the form of a tack (so called) or an arm. It has, however, been difficult to effect a satisfactory union between them and a base of iron or iron-containing metal. Moreover, such contacts have been subject to an excessive rate of wear and short life due to the heat produced at the point of contact which often causes the silver face plates to become pitted and rendered unfit for the purpose for which they are designed.

It is an object of the present invention to provide an electric contact of composite metal having a face plate of silver or silver alloy and a base plate of iron or iron-containing alloy that will be adapted to unite firmly with a tack or arm of iron or iron-containing metal.

It is a further object of the present invention to provide an electrical contact having a face plate of silver or silver alloy, which is easy to make and which stands up under long continued use.

Another object is to provide an argentic face plate for electrical contacts that is peculiarly adapted to be welded or otherwise firmly united to an arm or screw of ferric material.

Other objects of the present invention include the production of a composite sheet, bar or plate having a face plate of silver or silver alloy, an intermediate member of a metal or alloy of high conductivity, and a base layer of ferric metal, or alloy containing iron or nickel, each of the three metals or alloys being firmly and uniformly united to its adjacent layers.

The proportion and composition of the metals 55

or alloys of which the various members of my novel sheet are composed are so regulated and adjusted that the same is softer and easier to work than is the ordinary steel silver material and causes less wear on the tools used to form the ultimate contact members which are formed from it. The composite body of the present invention is so constructed that the silver and iron components thereof are very intimately joined together by a metal which has a strong affinity for argentic soldering or brazing material and for iron and silver as well. Consequently, the components of my novel electrical contacts are less apt to come apart than are ordinary contacts composed only of silver and steel, and in addition they last much longer by reason of the efficient conduction of heat away from the surface at which the heat is generated.

This conduction of heat is obtained through 20 the use of the intermediate layer of a metal of high heat conductivity which is so proportioned with relation to the other layers that it comprises between 15% to 35% by weight of the total composite body. The intermediate layer may be 10 as much as 40% of the total thickness of the composite body.

In general, the three metals or alloys are so 25 adjusted that none of them exceeds 50% of the total weight of the entire composition. Satisfactory material for the purpose may be constructed so that the various components fall within the following ranges by weight:

|                        | Percent  |
|------------------------|----------|
| Silver or silver alloy | 25 to 50 |
| Copper or copper alloy | 15 to 35 |
| Iron or iron alloy     | 50 to 15 |

The silver component of the composite body which represents the contacting surface proper may be either pure silver or sterling silver which 40 is about 92.5% silver and 7.5% copper, or may be coinage silver which consists of 90% silver and 10% copper, or it may be a different type of silver alloy. However, if the silver component is an alloy, the silver should exceed 50% thereof.

The intermediate layer of high heat conductivity may consist of pure copper or of copper alloy such as a copper-beryllium alloy or a copper-nickel alloy. If this layer is alloy, the amount of copper should exceed 50% of the total weight thereof.

The base layer may be pure iron such as Swedish iron or Armco iron or it may be an iron-nickel alloy. If it is an alloy, the iron should comprise more than 50% of the total.

In its simplest form the composite body of the

present invention may be illustrated by a contacting layer of pure silver, an intermediate layer of pure copper, and a base or bottom layer of Swedish iron, these three layers being united together by a thin film of silver solder. It is satisfactory to provide a starting material composed of a layer of silver metal having a thickness of .30 inch, an intervening layer of copper metal .20 inch and a third layer of Swedish iron of a thickness of .08 inch. Between each of the layers is inserted a thin layer of silver solder ranging from .002 inch to .004 inch in thickness.

The composite sheet of the present invention is produced by clamping the three metallic layers, together with the intervening strips of silver solder, with platers' clamps and placing the assembly into a suitable furnace, which is heated to a temperature sufficiently high to form a firm union between the metals with the silver solder. As will be hereinafter described, the assembly is subsequently worked down to a sheet of the desired thickness from which the ultimate contact members are formed.

As an example of a silver solder suitable for use in accordance with the present invention, the following is illustrative:

|        | Per cent |
|--------|----------|
| Silver | 60       |
| Copper | 30       |
| Zinc   | 8.2      |
| Tin    | 1.8      |

It should be understood that other suitable solders may be substituted for the silver solder provided that the same has a melting point lower than any of the melting points of the constituents of the composite body. The amount of the soldering composition should, of course, be only sufficient to cause a firm union between the constituent metals of the sheet.

The temperature of the furnace must be so adjusted that the assembled bar or composite sheet is brought to the point where the solder acts as a brazing material but should not be raised to a temperature at which the constituents of the bar or sheet are caused to melt or alloy with each other. The time of heating should not be prolonged so that the soldering or brazing metal is caused to seep out and run off from the seam between the constituent materials.

It should be understood that the union between the various constituents may be accomplished in an electric furnace, a gas furnace, or it may be electrically done by well known methods. It is preferable to carry out this operation in the presence of a reducing gas such as hydrogen.

After the composite sheet has been formed into a unitary mass, the same is removed from the furnace and allowed to cool, after which it is mechanically worked down by hammering, rolling, swaging, etc., until the desired thickness is obtained.

In the drawing, Fig. 1 illustrates in section a sheet or bar in which the above described metals or alloys have been firmly united. The layer 10 of silver is united to layer 11 of copper by a silver solder 13 of the nature described, and the said copper layer 11 is similarly united to an iron layer 12; Fig. 2 illustrates a contact member which has been punched out of the plate of Fig. 1 with a projection 14 on the steel end 13; Fig. 3 shows a steel or bimetallic strip 15 to which one of such contacts has been welded; and Fig. 4 shows a contact associated with a steel screw.

Instead of employing a brazing material of

the nature described, I may join the respective layers of my composite sheet together directly by welding, as by electric welding or by welding in a furnace, with or without the application of pressure. The welding operations are preferably carried out in an atmosphere of hydrogen at a temperature regulated to cause a welding or alloying of the respective surfaces without causing any appreciable melting of the constituent parts.

10 The process of the invention contemplates the combination of pressure with a temperature sufficiently high to make the metals plastic enough to cause them to flow and dissolve into one another. This is facilitated by working the metals in the manner previously described, except that they are rolled, swaged, etc., particularly during the first working operations, while they are relatively hot. This heat treatment during working may sometimes be found desirable in cases where the metals are brazed together as previously described, although it is not necessary in such cases.

When electrically welding the constituent metals, they may be placed between electrodes and sufficient pressure applied to the electrodes, as the current passes through them, so that the combined heat and pressure effects a perfect union of the nature described. It should be noted, however, that the current applied should be regulated so that the heat produced is not sufficient to bring the metals to their melting points.

35 The sheet may be processed into contact face plates of various shapes and sizes. It may be punched out into discs which may be circular, square, or of any convenient shape, adapted to be welded or brazed to suitable members such as metal arms, bimetallic members, metal plates, screws or rivets. For instance, if the disc is to

40 be used for spot welding, it may be extruded through rivet headers or other suitable machines to form small projections 14 on the steel or iron end of the composite member. These projections aid in permitting the contact to be more readily spot welded onto an iron or iron-containing arm or other suitable body to which it is to be attached. It may also be attached by its ferrous backing to a ferrous arm or tack by spot welding.

45 The component members of the present invention are very firmly and uniformly united together into a composite sheet which does not come apart under the most heavy use. The assembly is softer than the ordinary type steel and silver composition and causes less wear on the tools used to form the same into the desired contacts. The heat conductivity from the contacting surface is much greater than the ordinary form of contact by reason of the relatively large amount of material of high heat conductivity interposed between the contact surface and the base. The intermediate layer not only serves rapidly to conduct the heat away from the silver contact but it also serves to act as a cushion during processing, to give a strong bond between the silver and the steel, and to produce a superior contact.

50 It is a further advantage of the contact of this invention that by reason of the fact that the composite material of which it is composed provides a face plate of silver or silver alloy, an intermediate layer of copper or cuprous metal, and a backing of iron or ferrous metal, it is easily joined in a firm manner to iron-containing arms, rivets or the like. The contact of this invention

may, indeed, be easily spot welded to an arm of thermostatic bimetal where the side of the bimetal to which it is to be so welded consists of a nickel-iron alloy.

What I claim is:

1. A composite member consisting of a layer of argentic material, an intermediate layer of cupric material and a base layer of ferric material, the said intermediate layer comprising from 15% to 35% by weight of the composite member, and metallic means integrally uniting the same to the adjacent layers.

2. A composite member consisting of a layer of argentic material, an intermediate layer of cupric material and a base layer of ferric material, the said intermediate layer comprising from 15% to 35% by weight of the composite member and a substantial proportion of the total thickness thereof, and metallic means integrally uniting the same to the adjacent layers.

3. A composite member which consists of separate layers consisting, by weight, of 25% to 50% argentic material, 15% to 35% cupric material, and 50% to 15% ferric material, the said cupric layer being intermediate the other two and integrally uniting the adjacent layers together.

4. A composite member which consists of separate layers consisting, by weight, of 25% to 50% argentic material, 15% to 35% cupric material, and 50% to 15% ferric material, the said cupric layer being intermediate the other two layers and being intimately brazed thereto.

5. A tri-metallic member consisting of separate layers of argentic material and ferric material intimately joined to an intermediate layer of cupric material, the said intermediate layer comprising 15% to 35% by weight of the composite whole.

6. A tri-metallic electrical contact consisting of separate layers of argentic material and ferric material intimately joined to an intermediate layer of cupric material, the said intermediate layer comprising 15% to 35% by weight of the composite whole.

7. A composite metal member consisting of a layer of argentic material, an intermediate layer of cupric material, and a base layer of ferric material, the said intermediate layer comprising from 15% to 35% by weight of the composite member, and metallic means integrally uniting the same to the adjacent layers, said means comprising a silver solder.

8. A composite metal member consisting of a layer of argentic material, an intermediate layer of cupric material, and a base layer of ferric material, the said intermediate layer comprising from 15% to 35% by weight of the com-

posite member and a substantial proportion of the total thickness thereof, and a silver solder disposed between said respective layers whereby the same are integrally united to each other.

5 9. A composite material in the form of a sheet consisting of a layer of silver or silver alloy, a layer of iron or iron alloy, and an intermediate layer between the two said layers of copper or copper alloy comprising a relatively large proportion by weight of the thickness of the composite sheet, each of said three layers being integrally united to the next adjacent layer.

10 10. A composite metal member consisting of a layer of silver, an intermediate layer of copper, and a base layer of iron, the said intermediate layer comprising from 15% to 35% by weight of the composite member and comprising a substantial proportion of the total thickness thereof, and metallic means integrally uniting the same to the adjacent layers.

20 11. A composite metal member consisting of a layer of argentic material containing at least 50% silver, an intermediate layer of cupric material containing at least 50% copper, and a base layer of ferric material containing at least 50% iron, the said intermediate layer comprising from 15% to 35% by weight of the composite member and comprising a substantial proportion of the total thickness thereof, each of said layers being integrally united with the layer adjacent thereto.

25 12. A composite metal member consisting of a layer of argentic material containing at least 50% silver, an intermediate layer of cupric material containing at least 50% copper, and a base layer of ferric material containing at least 50% iron, the said intermediate layer comprising from 15% to 35% by weight of the composite member and comprising a substantial proportion of the total thickness thereof, each of said layers being united with the layer adjacent thereto by a thin metallic film having a lower melting point than any of said layers.

30 13. An electrical contact member comprising a layer of argentic material containing at least 50% silver, an intermediate layer of cupric material containing at least 50% copper, and a base layer of ferric material containing at least 50% iron, the said intermediate layer comprising from 15% to 35% by weight of the contact member and comprising a substantial proportion of the total thickness thereof, each of said layers being united with the layer adjacent thereto by a thin metallic film in a bond affording a good electrically conductive path throughout said contact member.

CLEMENS A. LAISE.